

BEST AVAILABLE COPY

# UNITED STATES PATENT OFFICE.

CARL MÖLLENHOFF, OF LEVERKUSEN, NEAR COLOGNE, GERMANY, ASSIGNOR TO  
FARBENFABRIKEN VORM. FRIEDR. BAYER & CO., OF ELBERFELD, GERMANY, A  
CORPORATION OF GERMANY.

## PROCESS OF DYEING AND PRINTING.

1,081,621.

Specification of Letters Patent. Patented Dec. 16, 1913.

No Drawing.

Application filed November 23, 1909. Serial No. 529,517.

To all whom it may concern:

Be it known that I, CARL MÖLLENHOFF, doctor of philosophy, chemist, citizen of the German Empire, residing at Leverkusen, 5 near Cologne, Germany, have invented new and useful Improvements in Processes of Dyeing and Printing, of which the following is a specification.

I have invented a new process of applying 10 reduction compounds of alizarin or its derivatives which contain in the center nucleus only one atom of oxygen characterized by the general formula:

15



20 in which the hydrogen atoms of the two outside nuclei may be substituted, for example by hydroxyl groups, to the fiber, thus producing very fast and deep shades on either the animal or vegetable fiber. Among these 25 substances I mention desoxyalizarin

30



desoxyflavopurpurin or desoxyanthrapurpurin with the formula:

35



40

and many others.

These reduction products produced from oxyanthraquinones may be applied directly to wool either in an acid dye-bath, or 45 in a bath containing a chromium mordant or they may be applied on chromed wool, while cotton is most advantageously dyed by being first chrome mordanted. The reduction products may also be employed for 50 printing in conjunction with pastes containing chrome mordants.

In carrying out my new process practically I can proceed as follows: Prepare a dye-bath containing 2 to 5 kilos of acetic

acid and 10 kilos of desoxyanthrapurpurin 55 (paste containing 20 per cent. of the dye). Enter 100 kilos of chromed wool, heat to boiling and boil during 1 to 1½ hours. A brilliant brown shade results. Desoxyflavopurpurin furnishes a deep brown. 60

Prepare a dye-bath containing 10 kilos of a 20 per cent. paste of desoxyflavopurpurin. Enter 100 kilos of chromed cotton yarn, heat the cold bath slowly to 80° C. and keep it at this temperature during some time. Dry, 65 steam, soap and dry. A deep brown is thus obtained which is fast to soaping.

Prepare a printing paste from 7½ kilos of a 20 per cent. paste of desoxyflavopurpurin, 7½ liters of chromium acetate (20° Bé.) and 70 85 parts of starch tragacanth thickening. Print upon oiled cotton cloth, dry, steam, soap and dry. A brown fast to soaping results.

Prepare a dye-bath containing 2 to 5 kilos 75 of acetic acid and 10 kilos of a 20 per cent. paste of desoxyalizarin, enter 100 kilos of wool at a temperature of 50 to 60° C., heat slowly to boiling and boil during ¾ to 1½ hours. A fast brown is thus obtained.

Prepare a dye-bath containing 10 kilos of a 20 per cent. paste of desoxyflavopurpurin acid and 2 to 5 kilos of acetic acid, enter 100 kilos of wool at 50° C., heat slowly to boiling and boil during 1 to 1½ hours. After cooling to 85 about 50 to 60° C. add 1 to 1½ kilos of bichromate of potassium and 1 kilo of acetic acid, heat to boiling and boil during ½ to 1½ hours. A very beautiful and fast brown is thus obtained. 90

Other of the above mentioned bodies may be used.

I claim:

1. The process of producing fast shades on textile fibers which comprises preparing 95 a dye-bath containing the reduction products of alizarin substances which contain in the central nucleus only one atom of oxygen, and in which products both keto groups have been reduced, immersing the fibers in said 100 bath, and fixing the dyes on the fibers by heating.

2. The process of producing fast shades on textile fibers which comprises preparing a 105 dye-bath containing the reduction products of alizarin substances which contain in the central nucleus only one atom of oxygen and which are substituted in the outside nuclei

- by hydroxyl, and in which products both keto groups have been reduced, immersing the fibers in said bath, and fixing the dyes on the fibers by heating.
- 5 3. The process of producing fast shades on textile fibers which comprises preparing a dye-bath containing the reduction products of alizarin substances which contain in the central nucleus only one atom of oxygen, 10 and in which products both keto groups have been reduced, immersing the fibers in said bath, and fixing the dyes on the fibers by heating in the presence of chromium compounds.
- 15 4. The process of producing fast shades on textile fibers which comprises preparing a dye-bath containing the reduction products of alizarin substances which contain in the central nucleus only one atom of oxygen, 20 and which are substituted in the outside nuclei by hydroxyl groups, and in which products both keto groups have been reduced, immersing the fibers in said bath, and fixing the dyes on the fibers by heating in 25 the presence of chromium compounds.
5. The process of producing fast shades on textile fibers which comprises treating the fibers with the reduction products of alizarin substances which contain in the central 30 nucleus only one atom of oxygen, and in which products both keto groups have been reduced, and fixing the dyes upon the fibers by heating in the presence of chromium compounds.
- 35 6. The process of producing fast shades on textile fibers which comprises treating the fibers with the reduction products of alizarin substances which contain in the central nucleus only one atom of oxygen, 40 and which are substituted in the outside nuclei by hydroxyl, and in which products both keto groups have been reduced, and fixing the dyes upon the fibers by heating in the presence of chromium compounds.
- 45 7. The process of producing fast shades on textile fibers which comprises mordanting the fibers with chromium compounds, treating the fibers with the reduction products of alizarin substances which contain in the central nucleus only one atom of oxygen, 50 and in which products both keto groups have been reduced, and fixing the dyes upon the fibers by heating.
8. The process of producing fast shades on textile fibers which comprises mordanting the fibers with chromium compounds, treating the fibers with the reduction products of alizarin substances which contain in the central nucleus only one atom of oxygen, 55 and which are substituted in the outside nuclei by hydroxyl, and in which products both keto groups have been reduced, and fixing the dyes upon the fibers by heating.
9. The process of producing fast shades on cotton fibers which comprises mordanting the fibers with chromium compounds, treating the fibers with the reduction products of alizarin substances which contain in the central nucleus only one atom of oxygen, 60 and in which products both keto groups have been reduced, and fixing the dyes upon the fibers by heating.
10. The process of producing fast shades on cotton fibers which comprises mordanting the fibers with chromium compounds, treating the fibers with the reduction products of alizarin substances which contain in the central nucleus only one atom of oxygen and which are substituted in the outside nuclei 65 by hydroxyl, and in which products both keto groups have been reduced, and fixing the dyes upon the fibers by heating.
- In testimony whereof I have hereunto set my hand in the presence of two subscribing witnesses.
- CARL MÖLLENHOFF.

Witnesses:

OTTO KÖNIG,  
CHAS. J. WRIGHT.

Correction in Letters Patent No. 1,081,621

It is hereby certified that in Letters Patent No. 1,081,621, granted December 16, 1913, upon the application of Carl Möllenhoff, of Leverkusen, near Cologne, Germany, for an improvement in "Processes of Dyeing and Printing," an error appears in the printed specification requiring correction as follows: Page 1, line 104, for the word "preapring" read *preparing*; and that the said Letters Patent should be read with this correction therein that the same may conform to the record of the case in the Patent Office.

Signed and sealed this 10th day of February, A. D., 1914.

[SEAL.]

J. T. NEWTON,

Acting Commissioner of Patents.

- by hydroxyl, and in which products both keto groups have been reduced, immersing the fibers in said bath, and fixing the dyes on the fibers by heating.
- 5 3. The process of producing fast shades on textile fibers which comprises preparing a dye-bath containing the reduction products of alizarin substances which contain in the central nucleus only one atom of oxygen, 10 and in which products both keto groups have been reduced, immersing the fibers in said bath, and fixing the dyes on the fibers by heating in the presence of chromium compounds.
- 15 4. The process of producing fast shades on textile fibers which comprises preparing a dye-bath containing the reduction products of alizarin substances which contain in the central nucleus only one atom of oxygen, 20 and which are substituted in the outside nuclei by hydroxyl groups, and in which products both keto groups have been reduced, immersing the fibers in said bath, and fixing the dyes on the fibers by heating in 25 the presence of chromium compounds.
5. The process of producing fast shades on textile fibers which comprises treating the fibers with the reduction products of alizarin substances which contain in the central 30 nucleus only one atom of oxygen, and in which products both keto groups have been reduced, and fixing the dyes upon the fibers by heating in the presence of chromium compounds.
- 35 6. The process of producing fast shades on textile fibers which comprises treating the fibers with the reduction products of alizarin substances which contain in the central nucleus only one atom of oxygen, 40 and which are substituted in the outside nuclei by hydroxyl, and in which products both keto groups have been reduced, and fixing the dyes upon the fibers by heating in the presence of chromium compounds.
- 45 7. The process of producing fast shades on textile fibers which comprises mordanting the fibers with chromium compounds, treating the fibers with the reduction products of alizarin substances which contain in the central nucleus only one atom of oxygen, 50 and in which products both keto groups have been reduced, and fixing the dyes upon the fibers by heating.
8. The process of producing fast shades on textile fibers which comprises mordanting the fibers with chromium compounds, treating the fibers with the reduction products of alizarin substances which contain in the central nucleus only one atom of oxygen, 55 and which are substituted in the outside nuclei by hydroxyl, and in which products both keto groups have been reduced, and fixing the dyes upon the fibers by heating.
9. The process of producing fast shades on cotton fibers which comprises mordanting the fibers with chromium compounds, treating the fibers with the reduction products of alizarin substances which contain in the central nucleus only one atom of oxygen, 60 and in which products both keto groups have been reduced, and fixing the dyes upon the fibers by heating.
10. The process of producing fast shades on cotton fibers which comprises mordanting the fibers with chromium compounds, treating the fibers with the reduction products of alizarin substances which contain in the central nucleus only one atom of oxygen and which are substituted in the outside nuclei 65 by hydroxyl, and in which products both keto groups have been reduced, and fixing the dyes upon the fibers by heating.
- In testimony whereof I have hereunto set my hand in the presence of two subscribing witnesses.
- CARL MÖLLENHOFF.

Witnesses:

OTTO KÖNIG,  
CHAS. J. WRIGHT.

Correction in Letters Patent No. 1,081,621

It is hereby certified that in Letters Patent No. 1,081,621, granted December 16, 1913, upon the application of Carl Möllenhoff, of Leverkusen, near Cologne, Germany, for an improvement in "Processes of Dyeing and Printing," an error appears in the printed specification requiring correction as follows: Page 1, line 104, for the word "preapring" read *preparing*; and that the said Letters Patent should be read with this correction therein that the same may conform to the record of the case in the Patent Office.

Signed and sealed this 10th day of February, A. D., 1914.

[SEAL.]

J. T. NEWTON,

Acting Commissioner of Patents.

It is hereby certified that in Letters Patent No. 1,081,621, granted December 16, 1913, upon the application of Carl Möllenhoff, of Leverkusen, near Cologne, Germany, for an improvement in "Processes of Dyeing and Printing," an error appears in the printed specification requiring correction as follows: Page 1, line 104, for the word "preapring" read *preparing*; and that the said Letters Patent should be read with this correction therein that the same may conform to the record of the case in the Patent Office.

Signed and sealed this 10th day of February, A. D., 1914.

[SEAL.]

J. T. NEWTON,  
*Acting Commissioner of Patents.*